

Sept. 8, 1942.

C. G. MUENCH

2,295,287

PACKAGE AND PACKAGING

Filed Jan. 10, 1938

2 Sheets-Sheet 1

Fig. 1.



Fig. 2.



Fig. 4.



Fig. 3.



Fig. 5.



Inventor:  
Carl G. Muench  
by Elmer A. Hampton  
Subj.

Sept. 8, 1942.

C. G. MUENCH

2,295,287

PACKAGE AND PACKAGING

Filed Jan. 10, 1938

2 Sheets-Sheet 2

Fig. 6.

EFFECT OF MOISTURE ON  
THREE WAY PACKAGED WASHER BAGASSE.  
ALL PACKAGES MADE AT SAME PRESSURE



Fig. 7.

THREE WAY PACKAGING OF WASHER BAGASSE  
MOISTURE 100%



Inventor:  
C. G. Muench  
by Edw A. Hampton

## UNITED STATES PATENT OFFICE

2,295,287

## PACKAGE AND PACKAGING

Carl G. Muench, New Orleans, La., assignor to  
The Celotex Corporation, Chicago, Ill., a cor-  
poration of Delaware

Application January 10, 1938, Serial No. 184,228

10 Claims. (CL 100—14)

This invention relates to the formation of compact self-sustaining packages of various materials, in particular relating to the formation of more or less disintegrated fibrous cellulose containing materials into such packages.

The shipment of such materials as sugar cane bagasse, the fibrous residue of sugar cane resulting from the processes of production of sugar, straw, corn stalks, fluffed paper, fiber, sawdust, extracted pine chips resulting from the extraction of turpentine from pine, raw cotton, straw, hay, oat hulls, kapok, and other like and more or less similar materials, are in many instances not economically feasible.

The economic bar to transportation of the above materials and similar materials arises due to their bulk since the weight of the various materials mentioned runs generally from about 2 to 6 lbs. per cubic foot and as it will be readily understood the bulk of materials of such low density is so great that transportation of materials of such densities other than over very short distances is not economical. The economic bar to the transportation of such materials applies particularly to those of the above mentioned materials which are of least value such as sugar cane bagasse, sawdust, extracted pine chips and other comparable materials.

It is a particular object of this invention to disclose a manner for packaging materials of the general character above enumerated in such manner that these materials when packaged may be economically transported for fairly long distances. Incidental to the particular object of this invention, further objects of the invention are the formation of such packages at a high density, having coherence and especially having the property of being readily disintegrated when desired.

Packaging of materials of the general class enumerated, at high density, places them in a condition for economical transportation in which connection investigation discloses that rail and ship freight rates are such that packages of these materials having a density of around 45 to 50 lbs. per cubic foot are of an economic density. Coherence of the packages is of extreme importance in that if the packages must be secured with heavy steel bands such as are used to secure the ordinary dense supercompressed export bales of raw cotton, this constitutes a severe handicap economically. The packages formed in accordance with the teachings of this invention have such coherence that either no restraining means or only very light restraining means are required,

more for surface protection than for any other reason as for example the formed packages of the more valuable materials such as cotton and kapok may advisedly be covered with burlap and lightly banded.

Packages of materials formed in accordance with the teachings of this invention, it has been discovered, may be readily disintegrated with very surprising rapidity. On placing one of these high density bales in water, preferably warm water, the water is very quickly absorbed and the package rapidly swells and expands three dimensionally and moisture is quickly absorbed throughout the material. A package of bagasse fibers formed in accordance with the teachings of this invention and having a density of between 45 and 50 lbs. per cubic foot and of dimensions 4" x 4" x 4" was completely saturated and disintegrated to substantially the condition of the bagasse before formation into the package in a period of approximately two minutes after submerision in warm water. The same weight of package compressed into a package by ordinary baling methods, one dimensional compression, of about five times the volume or with a density of about 10 lbs. per cubic foot when similarly placed in warm water was not completely saturated and disintegrated in a period of several hours. It is to be understood that in the comparison above given, there was no agitation in either case since, of course, the low density package could have been readily broken up by stirrers or the like and have been caused to become rapidly saturated through continued agitation.

The objects of this invention are achieved by three-way compression, of the materials mentioned, in the procedure of packaging and in the drawings accompanying this specification, the apparatus for accomplishing such compression is shown, together with illustrations showing the various steps of formation of a package. Also in the drawings there are shown several curves illustrating the relationship between various factors involved in the production of a satisfactory package produced in accordance with the invention herein disclosed. In the drawings; Figure 1—is a diagrammatic perspective of the packaging apparatus employed; Figure 2—is a perspective illustrative of the original volume and relative dimensions of the material to be packaged; Figure 3—is a perspective of the volume and relative dimensions of the material after the first step of packaging; Figure 4—is a perspective of the volume and relative dimensions of the

material after the second step of packaging; Figure 5—is a perspective of the volume and relative dimensions of the material after the third step of packaging; Figure 6—is a curve showing the relationship between density of the package formed plotted against the moisture content of the material to be packaged; and Figure 7—is a curve illustrating the relationship between the density of the package formed plotted against the pressure used in the final step of compression.

In describing the invention hereof the specific description given will be based upon the formation of a finished package having dimensions of approximately 4" x 4" x 4" formed from washer bagasse. This limitation of the specific description is made due to the fact that more data has been accumulated in this particular connection than with respect to the packaging of any other specific material or other size of finished package.

Washer bagasse, as the term is herein used, refers to sugar cane bagasse which results from the usual operations of crushing sugar cane for the recovery of the cane juice therefrom as generally practiced in the production of sugar in Louisiana which bagasse has been further treated as hereafter described. The sugar cane bagasse produced resulting from the production of sugar is baled in a baling machine which is similar to the ordinary baler used for the baling of straw, hay, and the like, except that it is somewhat more massively built, the bales produced thereby being substantially similar to the ordinary bale of hay, or straw. These bales are stored under conditions which bring about a limited retting of the bagasse as disclosed in the patent to Elbert C. Lathrop et al., No. 1,633,594. This retted bagasse is subjected to a cooking with water at a steam pressure of about 50 lbs. per square inch for about 45 to 60 minutes, is then removed from the cooker, run through a swing hammer shredder and washed with water to constitute washer bagasse. This washer bagasse, dried but loose, that is, not compressed, has a density of about 3 to 4 lbs. per cubic foot.

In the formation of packaged washer bagasse in accordance with this invention, washer bagasse is loaded loosely into compression apparatus 10 which is substantially a cubical chamber having very strongly constructed walls 14 with plungers 11, 12 and 13 each of which operate through various faces of the walls 14. Before the chamber defined by the walls 14 is loaded with the washer bagasse, plunger 11 is entirely withdrawn and plungers 12 and 13 are withdrawn until the inner faces are flush with the interior of the frame 14 of the apparatus. The interior dimensions of frame 14 are, in the particular apparatus being described, 12" x 12" x 12" and an 8" depth of the washer bagasse is introduced into the chamber to the end that approximately 2 lbs. of washer bagasse are introduced as a mass having dimensions 8" x 12" x 12" corresponding to dimensions A, B and C respectively, Figure 2. Plungers 12 and 13 are suitably anchored in their withdrawn positions as by pins inserted through registering openings in the respective plungers and frame 14, such openings and pins not being shown as the arrangement thereof is obvious and would only tend to obscure the showing in the drawings. Plunger 11 is then inserted into the opening of the upper face of the frame work 14 as shown

in Figure 1 and is forced downwardly by appropriately applied pressure.

It is to be understood that plungers 11, 12 and 13 are operated by suitable operating means, as by pressure cylinders or the like, suitably connected thereto. In experimental work done, the plungers were forced inwardly by suitably positioning the frame 14 and plunger to be forced inwardly between the upper and lower faces of a hydraulic press. In the press used and under conditions as above described, plunger 11 was forced downwardly a distance half of the dimension A to the dimension A' compressing the charge of washer bagasse down to the dotted line shown in Figure 2. The total force applied to plunger 11 was difficult to read on the gauge of the press but it was estimated that there was applied to plunger 11 a force of between 1 and 2 tons which, being applied on the surface of the charge 12" x 12", resulted in a pressure of between 1 and 2 tons per square foot, being exerted on the charge during this step of the compression. The pressure to be applied at this stage of the compression will of course vary somewhat, particularly in packaging different materials but the figures given are indicative.

When plunger 11 is forced in to compress the charge to the dimension A', it is secured by suitable means such as by pins and registering holes, not shown, provided in the frame 14 and plunger 11, and then the next operation may proceed. Pressure is applied to plunger 12 to force it inwardly, the pins previously mentioned as holding this plunger having, of course, been removed before the pressure is applied, and sufficient pressure is applied to compress the charge from the dimension B to the dimension B', as shown in Figure 3 of the drawings, the dimension B' being 4". On the gauge of the press used the actual pressure applied was difficult to determine but pressure on the plunger appeared to be in the range of from 2 to 4 tons or at the rate of from around 5 to 10 tons per square foot. After plunger 12 was forced inwardly to compress the charge down to the dimension B' as shown by the dotted line in Figure 3, this plunger was suitably secured in position as described in connection with the securing of plunger 11.

As the next step of the process, the plunger 13 was forced inwardly, the pins holding this plunger in withdrawn position, having of course been removed before the pressure was applied, and plunger 13 was forced inwardly sufficiently to compress the charge from dimension C to a dimension somewhat slightly less than dimension C' being, for the particular apparatus shown, 4". On the compression the gauge pressure on the press ranged between 32 and 40 tons, being held as nearly as possible to 35 tons, which being applied on a face 4" x 4" in dimension, that is, an area of 16 square inches, amounted to a pressure of between 2 and 2½ tons per square inch, averaging about 2½ tons per square inch.

Plungers 11, 12 and 13 were then released and removed from frame 14 and the resulting densely compressed packaged washer bagasse with dimensions of approximately 4" x 4" x 4" was removed. The packaged washer bagasse, providing the proper moisture content was present at the beginning of the compression as will be hereinafter discussed, and compressed at a final pressure of from 2 to 2½ tons per square inch, will have on removal from the apparatus a density of about 48 lbs. per cubic foot which, overnight, will drop to about 43 lbs. per cubic foot

and may in a week or so drop further to about 40 lbs. per cubic foot, after which lapse of time the density apparently does not further decrease, that is, the package has no further expansion.

The moisture content of the charge, when the compression begins, is very important in determining the density of the package when finally compressed and in achieving the desired cohesion so that a firm package which may be handled and shipped will result from the procedure as above described. For washer bagasse the preferred moisture content of the charge when placed in the frame for compression has been found to be a moisture content of approximately 11% based on the weight of the dry fiber and in this connection reference is made to Figure 6 of the drawings. If the initial moisture content is the optimum as shown in Figure 6, that is, 11%, the density with a final pressure of approximately 2 tons per square inch is the maximum and regain or expansion overnight is a minimum. It is, of course, to be understood that although a moisture content of 11% is the optimum, reasonable variation therefrom is allowable and will produce a satisfactory package as may be seen from Figure 6 which shows that a satisfactory package can be made if the material as charged has a moisture content of from about 5 to 15%, or if a final package of a somewhat lower density will serve, the moisture of the charge may be outside of the approximate limits above noted, say between about 3 to 18%.

Reference to Figure 7 shows that on increasing the pressure for a given moisture content of charge there will result a finished package of increased density. By combining the teachings of Figures 6 and 7, it is obvious that if for some reason it is necessary that the finished package have a high density, the desired increased density may be obtained for a given initial moisture content of the charge by raising the pressure per square inch of the final pressing. As shown in Figure 7 for washer bagasse of 10% initial moisture content, the density of the finished package may be raised from 44 to 51 lbs. per cubic foot by raising the final pressing pressure from 1.87 tons to 2.5 tons per square inch, or if a lower density will suffice, for a given moisture content, in this case 10%, a lesser pressure may be used on final pressing as shown, a pressure of 1.25 tons per square inch resulting in a package having a density of about 41 lbs. per cubic foot. It appears that excessive pressure on final compression tends to injure the fiber and therefore it is suggested that in no case should pressure exceeding 5 tons per sq. in. be applied, this is of course subject to determination for any particular material and when working with any particular material the upper allowable limit of pressure practical may be readily ascertained.

Procedure similar to that above described has been employed in packaging numerous materials other than washer bagasse, the material concerning which detailed description of the procedure was given. Among the various other materials packaged in accordance with the teachings of this invention are raw bagasse, that is, bagasse which has not been cooked but instead has only been shredded, spent pine chips, fluffed kraft fiber, fluffed sulphite fiber, kraft lap, kapok and sieved raw bagasse. The experiments made with the various materials just mentioned, which experiments were carried on in considerable detail together with less extensive experiments made with other more or less like and similar substances

have clearly indicated that the method of packaging disclosed herein is applicable to cellulosic materials generally, including such materials as all of the usual paper making fibers, including such materials as cotton, flax, hemp, ramie, etc., and is also applicable to other less known materials such as peanut hulls, bean pods, rice, wheat, and oat hulls and other materials.

In the experimental procedure of packaging various of the materials particularly above mentioned, the procedure followed substantially is that hereinbefore specifically set out but with some exceptions as will be hereafter noted. In the packaging of kraft lap which is a rather loosely felted fiber sheet the structure of which may be said to be roughly comparable to that of a loosely sheeted blotting paper, since this material is already of considerable density having had in its formation what is substantially the equivalent of the first compression of the packaging process hereof, this material was loaded into the compression apparatus to a depth of only about 3", and the first compression step was not in fact a compression of the kraft lap material since the plunger 11 was brought down only to its normal position, that is, to within 4" of the bottom of its stroke. On the second stroke, when plunger 12 was forced inwardly, the kraft lap material was of course re-arranged and compressed into the second phase of the compression operation and then the final compression by means of plunger 13 was carried out in the usual manner.

In the experiments involved in the packaging of kapok, it was found that the compression apparatus should be filled with kapok to approximately its full height after which the various compressive steps were carried out in the described manner. It was noted that the kapok package was not quite so firmly knit and integrated as were the other materials when packaged in accordance with the procedure of this invention but it appeared that this was due to the fact that the experimental apparatus which was being used was limited in the pressure which could be applied to the plunger 13 for the final compressive step and all indications of the experiment were to the effect that had it been possible to increase the pressure on the last stage of the compression, the kapok package would have been as satisfactory as the packages of the various other materials used.

The sieved bagasse experiments were made with material comprising raw bagasse which had been shredded in a swing hammer shredder through plates having  $\frac{1}{8}$ " holes and subsequently sieved through a 30 mesh screen, the portion which was used in the experiment being the fine portion of such material which passed through the 30 mesh sieve. This sieved material, which was only very finely fibrous settles relatively solidly due to the fine subdivision so that the mere act of loading the material into the chamber of the compression apparatus results in a compacting which is substantially the equivalent of the first step of compression of the process as applied to a more coarsely fibrous material and has a density of approximately 6 lbs. per cubic foot so that this material was loaded into the compression apparatus to the extent of only about 4" in depth. When plunger 11 was brought down, of course the material in the apparatus was compressed only slightly and after this step of the operation the two following compressions were carried out in the usual manner. This sieved bagasse, due

to its fineness, produced a block which out of the press had a density of 58 lbs. per cubic foot but which overnight dropped to a density of about 52 lbs. per cubic foot, thereafter remaining substantially constant.

Experiments generally similar to those above described were carried on to produce finished packages having dimensions 1" x 1" x 1" and it was found that various phases of these experiments were substantially similar to those of the experiments above described in detail except that on the final stage of the compression, pressures ranging from 2 to 3 times as great were required to obtain the same final results. The necessity of the use of the considerably higher final pressures is attributed to the fact that in the apparatus used in producing the finished 1" cubical packages, the ratio of the frictional surfaces with respect to the area of the face against which the plunger is operating is considerably higher than in the larger apparatus whereby the frictional resistance is much greater thus necessitating the use of higher pressures to accomplish equivalent final results.

A similar line of experiments was carried out on a large press producing a finished package having dimensions approximately 14" x 14" x 14". In experiments with this press using retted but not cooked bagasse, the frame which had internal dimensions 42" x 48" x 52" was filled approximately one-third full with bagasse, and the respective strokes of the plungers in three directions, each at right angles to the other, were made in sequence as described in connection with the production of packages in the form of 4" cubes, and with a pressure of about between 2½ and 3 tons per square inch on the final stroke, finished integrated and firmly coherent packages were produced having a density in the neighborhood of 48 lbs. per cubic foot.

Generally speaking the experiments made, taken as a whole, indicate that the successive compressions should reduce the volume of the material in the apparatus about as follows:

On the first compression, up to 50%.  
On the second compression—50 to 70%, optimum about 66%.  
On the third compression about 60 to 80%, optimum 70 to 75%

it, of course, being understood that on the third compression there is a regain on the release of the plunger pressure so that the actual final reduction in volume is in the neighborhood of 66%. The pressures required are about 0 to 1 ton per sq. ft. of surface on which pressure is applied in the first compression but with a possible range of 0 to 5 tons per sq. ft.; about 2 tons per sq. ft. of surface on which pressure is applied in the second compression with a possible range of 2 to 10 tons per sq. ft.; and 2 to 3 tons per sq. in. of surface on which pressure is applied in the final compression with a possible range of 1.5 to 5 tons per sq. in. All of these general figures just above given, it is to be understood, are approximate and for the best results with any particular material, the values as given must be appropriately digressed from to the preferred values which can only be accurately determined for a particular material by experiments made in accordance with the detailed description hereinabove set out, although as has been indicated, the values given as comprising the general fig-

ures applicable produced in all cases reasonably satisfactory finished packages.

It is to be understood that for the purpose of speeding up the operation for forming packages as hereinabove described or as a matter of convenience in transporting the material to be packaged from the source of supply to the packaging operation, it may be convenient or advisable to bale the materials in more or less conventional manner, in which case it is preferable that the bales be made to conform to the conditions which would result from the first step of the packaging operation as described, whereupon such bales may be placed directly into the packaging machine, with plunger 11 locked at the inner end of its normal stroke whereupon the second and third compressions can then be carried out in sequence in accordance with the above described procedure.

The action of the packaging as above described is believed to be that in the first stage of the compression, the relatively loosely arranged fibers are compacted and pushed together along the axis in the direction in which the compression is applied, then when the second stage of compression is applied, these fibers are again compacted and pushed together along an axis at right angles to the original axis of the first compacting and finally in the third stage of the compression, the fibers are compacted and pushed together in the direction of a third axis which is at right angles to each of the axes previously mentioned so that the net result is that the fibers are successively pushed together and compacted from each of three directions, each at right angles to one another and therefore the fibers are caused to firmly interweave and interlock under the pressure of the final compression, such interweaving and interlocking being to such an extent that they are held together by the frictional contact of the fibers to the extent that an integrated dense handleable package is produced.

It is to be understood that the above description is illustrative of the invention and that the such description is not to be taken as limiting the application of the invention but that it is given only for the purpose of teaching the procedure to be followed in packaging materials of the character of the materials which have been specifically mentioned and that those skilled in the art, to which this invention appertains, will readily understand from the above description the procedure which should be followed in determining the preferred values to be used in forming materials other than those specifically described into dense integrated and self-sustaining packages having the most desirable characteristics.

Having disclosed and described my invention in detail, I claim:

1. The process of forming fibrous bagasse and like substances with 3 to 18% moisture content into hard and dense self-sustaining unit packages comprising charging the substance into a container, compressing the substance in the direction of the axis to the applied compressive force, then while the material is held under such compressive force applying thereto a second compressive force applied at a right angle to axis of the first compressive force and finally while held under the action of the previously applied compressive forces subjected to a further compressive force applied in a direction at a right angle to each of the previously applied compressive forces, each compres-

sion force increasing in intensity to effect final compression of the substance to a density in excess of 50 lbs. per cubic foot and upon release of pressure in excess of 30 lbs. per cubic foot.

2. The process as defined in claim 1 wherein the successive compressions are by volume respectively approximately 50, 66½ and 75% of the respective volume of the material at the start of each of the successive steps of compression.

3. The process as defined in claim 1 wherein the substance as charged into the container has a density of between 2 and 4 pounds per cubic foot and a moisture content of between 5 and 15%, based on dry weight of the substance, the first compression is at a pressure of between 0 to 5 tons per square foot of surface against which the compressive force acts the volumetric compression being about 50% of the original volume, the second compression is at a pressure of between 2 to 10 tons per square foot of surface against which the compressive force acts the volumetric compression being about 66½ % of the volume at the beginning of the second step of compression, and the third compression is at a pressure of between 2 to 5 tons per square inch of surface against which the compression force acts the volumetric compression being between 60 to 80% of the volume at the beginning of the third step of compression.

4. The process of integrating a mass of fibrous cellulosic substance having 3 to 18% moisture content into a dense, self-sustaining package by successive steps of compacting in three directions, each direction of compacting being at right angles to each of the other directions of compacting and each of the successive compactings increasing the density of the mass to a final compressed density, while under compression of compacting, of substantially 60 lbs. per cubic foot for the integrated mass.

5. The process of producing a dense, self-sustaining package of cellulosic substance wherein a mass thereof having a moisture content of between 3 and 18% is compressed in the direction of an axis of compression to a volume of about one-half of the original mass, then compressed in the direction of an axis of compression at right angles to the first axis of compression to a volume of about one-third the last previous volume and finally compressed in the direction of an axis at right angles to each of the previous directions of compression to a volume of about 25 to 33% of the volume of the mass previous to the last compression.

6. A mass of fibrous cellulosic substance having a moisture content of between 3 and 18% based on dry weight of the mass, integrated by at least three successive compactings, each acting at substantially right angles to the preceding compacting causing a self-sustaining package of density in excess of 30 lbs. per cubic foot to be formed.

7. A new article of commerce comprising bagasse fiber integrated by subjection, while having

a moisture content of between about 3 to 18%, to successive steps of compression, each such succeeding step being at substantially right angles to each of the other directions of compression and each successive compression applied being of increasing intensity, a succeeding compression applied to the fiber while held confined and subjected to the preceding compression step and steps respectively, the fibers thereof interlaced and interwoven to a density of not less than 30 lbs. per cubic foot and forming a hard, dense, commercially economic unit package which is self-sustaining.

8. A self-sustaining cellulosic fiber block comprising a unit mass of intertwined and overlapping fibrous substances of vegetative origin interlaced in such close proximity to each other that the density of the mass is not less than 30 lbs. per cubic foot, such density being obtained by the application to a substantially loose mass of such fibrous substances having an initial density in excess of about 4#/cu. ft. and a moisture content of between 3 to 18% based on the dry weight of the mass of non-percussive pressure applied successively and with successively greater intensity of pressure per unit area to which applied from three independent sources applied respectively at right angular directions of application to the mass, the mass being continuously confined; the first application of non-percussive pressure compressing the mass to a volume of substantially one-half of the original mass, the second application of non-percussive pressure compressing the mass to a volume of about one-third of the last previous volume, and the final application of non-percussive pressure compressing the mass to a volume of one-fourth to one-third of the volume of the mass previous to the application of the final application of the pressure.

9. An integrated and self-sustaining package of cellulosic fibers, the moisture content thereof between about 3 per cent to 18 per cent and the density thereof in excess of 30 pounds per cubic foot, the density throughout the mass being substantially uniform and the fibrous structure thereof of interlaced and frictionally interlocked throughout, predominantly in three planes and resulting from three successive compressions of increasing intensities applied each at right angles to each of the others.

10. A self-sustaining cellulosic fiber block comprising a mass of cellulosic fibers of a moisture content of between 3 per cent to 18 per cent, the fibers thereof throughout frictionally interlaced and overlapped and resulting from the compression of the mass thereof by successive and different compressions applied from three independent sources, each acting in a plane at right angles to each of the others, the density of the block throughout being in excess of 30 pounds per cubic foot.

CARL G. MUENCH.